

# United States Patent

[11] 3,619,284

|                |                                                                                                                       |                                                                                                                                                                                                                                                      |                                       |
|----------------|-----------------------------------------------------------------------------------------------------------------------|------------------------------------------------------------------------------------------------------------------------------------------------------------------------------------------------------------------------------------------------------|---------------------------------------|
| [72] Inventors | Dilip K. Ray-Chaudhuri<br>Somerset;<br>Stanley Field, Piscataway; Irving D.<br>Hodgkin, Neshanic Station, all of N.J. | [50] Field of Search.....                                                                                                                                                                                                                            | 117/201,<br>154, 218, 76, 86; 162/138 |
| [21] Appl. No. | 816,777                                                                                                               | [56] References Cited                                                                                                                                                                                                                                | UNITED STATES PATENTS                 |
| [22] Filed     | Apr. 16, 1969                                                                                                         | 3,264,137                                                                                                                                                                                                                                            | 8/1966 Gess..... 117/201              |
| [45] Patented  | Nov. 9, 1971                                                                                                          | 3,335,100                                                                                                                                                                                                                                            | 8/1967 Geyer..... 117/201 X           |
| [73] Assignee  | National Starch and Chemical Corporation<br>New York, N.Y.                                                            | 3,348,970                                                                                                                                                                                                                                            | 10/1967 Gess..... 117/201             |
| <hr/>          |                                                                                                                       |                                                                                                                                                                                                                                                      |                                       |
| [54]           | <b>ELECTROCONDUCTIVE PAPER AND PROCESS<br/>OF MAKING SAME</b><br>8 Claims, No Drawings                                | <i>Primary Examiner—William L. Jarvis<br/>Attorney—Thomas B. Graham</i>                                                                                                                                                                              |                                       |
| [52]           | U.S. Cl.....                                                                                                          | <b>ABSTRACT:</b> A paper having a surface adapted for electrostatic printing and a process for preparing such paper; said paper containing at least one monoquaternary nitrogen compound which serves as the electrostatic electroconductive medium. |                                       |
| [51]           | 117/201,<br>117/76, 117/86, 117/154, 117/156<br>Int. Cl..... G03g 5/00                                                |                                                                                                                                                                                                                                                      |                                       |

ELECTROCONDUCTIVE PAPER AND PROCESS OF  
MAKING SAME

## BACKGROUND OF THE INVENTION

This invention relates to novel, electrically conductive paper which is useful in the electrostatic printing art. It relates more particularly to paper having a coated surface adapted for electrostatic printing and which contains at least one monoquaternary nitrogen compound which serves as the electrostatic electroconductive medium. In a further aspect, the invention relates to the process of making the thus described paper.

In electroconductive printing processes the treated surface of the electroconductive paper is subjected to a modulated voltage in a predetermined pattern. The thus-imparted electrostatic charge produces a latent image in accordance with the intensity of the applied voltage. The latent image is subsequently made visible, ordinarily by the application of a powdered reagent carrying a charge opposite to that of the electrostatic charge on the paper; the latter powder being permanently fused to the paper upon being heated or by other selected means. A particular shortcoming of many conductive media which are presently used to produce electroconductive paper lies in their diminished ability to remain conductive in a dry atmosphere, i.e. at relative humidities ranging below about 50 percent.

Broadly stated, it is a primary object of this invention to provide improved, electrically conductive coated paper which is useful in electrostatic printing processes under all ambient conditions including conditions of low relative humidity.

Another object of this invention is to provide electrically conductive coated paper having a surface resistivity, i.e. the reciprocal of conductivity, of from about  $4 \times 10^5$  to  $2 \times 10^9$  ohms/cm.<sup>2</sup> at relative humidities ranging from about 25 to 50 percent; the latter resistivity values being required in any paper which is to be successfully used in electroconductive processes.

Other objects and advantages of our invention will be made apparent from the following description.

## SUMMARY OF THE INVENTION

We have now discovered that when certain monoquaternary nitrogen compounds are coated upon, or otherwise introduced, to a paper substrate so as to provide an electrostatic printing surface, the aforementioned objects are all readily achieved. Furthermore, the use of these specified monoquaternary nitrogen compounds does not, surprisingly, require the coincident use of deliquescent salts, such as lithium or zinc chlorides, as was previously thought to be necessary in order to impart a satisfactory level of conductivity with a given concentration of a quaternary ammonium compound. (See, for example, U.S. Pat. Nos. 3,264,137 and 3,348,970).

The monoquaternary nitrogen compounds suitable for use in the present invention are those which correspond to the following structural formulas:



wherein R is an alkyl group containing from one to 22 carbon atoms; R' is a radical selected from the group consisting of alkyl, aryl, aralkyl, cycloalkyl, halo-alkyl, halo-alkenyl, halo-alkylyl, HOCH<sub>2</sub>CHOHCH<sub>2</sub>-, H--OCH<sub>2</sub>CH<sub>2</sub>-, and



groups wherein n may have a value of from 0 to 19; A is an alkylene radical containing from two to seven carbon atoms; X is an alkyl group containing from five to 15 carbon atoms; and Y is an anion selected from the group consisting of the chlorine, bromine, iodine, methosulfate and ethosulfate anions.

The monoquaternary nitrogen compounds useful in the process of this invention are relatively soluble in water, and generally exhibit indeterminate melting points. These compounds are either available commercially or methods for their preparation may be found in the literature.

Among the monoquaternary nitrogen compounds represented by the foregoing structural formulas are:

Group 1. 2-Undecyl-1-methyl-1-hydroxyethyl-1,4,5-dihydroimidazolinium chloride and 2-Heptadecyl-1-methyl-1-hydroxy-propyl-1,4,5,6-tetrahydropyrimidinium methosulfate,

Group 2. N-Isopentadecyl-N-trimethyl ammonium chloride and N-Isoundecyl-dihydroxyethyl-methyl ammonium chloride,

Group 3. N'-Dodecanoyl-N,N-dimethyl piperizinium chloride,

Group 4. N-Dodecyl-methylpyrrolidinium chloride,

Group 5. N-Tetradecyl-methyl piperidinium chloride,

Group 6. 2-Hydroxy-3-dodecyl benzyl trimethyl ammonium chloride,

Group 7. N-Hexadecyl-ethyl morpholinium ethosulfate,

Group 8. 1,2-trimethylene-1-decyl-1,4,5,6-tetrahydropyrimidinium bromide,

Group 9. N-Dodecanamidopropyl-trimethyl ammonium chloride,

Group 10. Dodecyl trimethyl ammonium chloride, Tallow (C<sub>14</sub>-C<sub>18</sub>) trimethyl ammonium chloride and Tallow (C<sub>14</sub>-C<sub>18</sub>) dimethyl chloro-2-butetyl ammonium chloride.

With respect to the concentration of the monoquaternary nitrogen compound which is required in the resulting electroconductive paper, ordinarily, one or more of these compounds should be applied onto a paper substrate so that the thus treated paper contains the monoquaternary nitrogen compound in a concentration of from about 0.5 to 6 pounds per ream (3,000 sq. ft.). An effective degree of conductivity for most electroconductive purposes is achieved with paper containing from about 2 to 5 pounds of the selected compound per ream. The use of an increased concentration of the monoquaternary nitrogen compound, while producing increased conductivity, will, of course, result in increased production costs.

A variety of procedures may be used to prepare the improved electroconductive paper of this invention. For example, in a preferred embodiment, an aqueous solution of the selected monoquaternary nitrogen compound, or a mixture thereof, is admixed with a conventional polymeric coating

material, ordinarily in the form of an aqueous dispersion, and the resulting blend is then applied to the paper substrate by coating, dipping, spraying, or any other technique that can be utilized for the application of an aqueous coating system onto a paper substrate. Suitable polymeric coating materials include any aqueous based polymeric material of a type ordinarily used for coating paper stock that is to be employed in electroconductive processes but which are, however, compatible with the selected monoquaternary nitrogen compound. Examples of such polymeric coating materials include: (1) polyvinyl acetate and the random copolymers of vinyl acetate with one or more monomers selected from the group consisting of: (a) the alkyl esters of acrylic and methacrylic acid, wherein said alkyl group contains from one to about 10 carbon atoms, such, for example, as methyl acrylate, butyl acrylate, 2-ethylhexyl acrylate, and the corresponding methacrylate esters; (b) vinyl and vinylidene halides, such, for example, as vinyl chloride and vinylidene chloride; (c) ethylenically unsaturated monocarboxylic acids, such, for example, as acrylic, itaconic, citraconic, and crotonic acids; (d) nitriles of ethylenically unsaturated monocarboxylic acids, such, for example, as acrylonitrile; (e) ethylenically unsaturated dicarboxylic acids, such, for example, as maleic and fumaric acid; (f) anhydrides of ethylenically unsaturated dicarboxylic acids, such, for example, as maleic anhydride; (g) the C<sub>1</sub>-C<sub>4</sub> alkyl esters of maleic and fumaric acid, such, for example, as methyl hydrogen maleate; and, (h) the dialkyl esters of ethylenically unsaturated dicarboxylic acids, wherein said alkyl group contains from one to about eight carbon atoms, such, for example, as dibutyl maleate; (2) polyvinyl alcohol; (3) amylose-based materials such as starches; starch derivatives such as esters and ethers of starch; and, starch conversion products such as oxidized starches and dextrins; and (4) cellulose derivatives such as methyl cellulose, ethyl cellulose, hydroxyethyl cellulose and hydroxypropyl cellulose. Mixtures of any two or more of the latter coating materials can also be used if desired.

The compositions may, if desired, contain a variety of optional ingredients in order to modify certain properties of the resulting compositions. Such ingredients include, for example, pigments, defoamers, fillers, and the like.

Ordinarily, the concentration of the monoquaternary nitrogen compound in the coating blend is from about 4 to 40 percent, by weight, of the resulting blend. The proportion of polymeric coating material solids in the blend may ordinarily vary from about 5 to 50 percent, by weight, of the resulting blend. The total solids content of the blend should be in the range of from about 10 to 70 percent, by weight.

After coating the paper substrate with the above described coating blend, the paper is ordinarily dried by means of any convenient procedure such, for example, as by passing over a drying roll or by the use of an oven. The properties of the resulting coated paper can be modified, as desired, by varying the concentration and/or the particular type of polymeric coating material which is utilized.

The electroconductive paper of this invention may also be prepared by means of a procedure wherein an aqueous solution of the monoquaternary nitrogen compound is applied to the paper substrate by coating, dipping, spraying, or any other selected means. The concentration of the monoquaternary nitrogen compound which is present in the aqueous solution is not critical and may be varied, as desired, provided that the latter compound is present in the resulting electroconductive paper in a concentration of from about 0.5 to 6 pounds per ream. After being dried, the paper prepared in this manner may subsequently receive an additional coating or sizing of a polymeric material of the type described hereinabove.

In another variation of the process of this invention, an aqueous solution of the selected monoquaternary nitrogen compound can be applied to paper which has previously been coated with a polymeric coating material. Thus, in this procedure, the polymeric coating material, selected from the polymeric coating materials described hereinabove, is applied

to the paper whereupon it is dried and the conducting coating is subsequently applied to the surface of the substrate which has received the polymeric coating.

In still another variation of the process of this invention, those paper substrates having a dense, so-called tight surface may be coated with an aqueous solution of the monoquaternary nitrogen compound without the subsequent application, thereto, of a polymeric top coat. For example, an aqueous solution of a monoquaternary nitrogen compound need merely be applied onto the surface of such a substrate whereupon, after being dried, it is ready for use.

It is to be noted that any type of paper stock may be utilized as the substrate material for the novel electroconductive papers of this invention. Further, if desired, the electroconductive paper resulting from any of the above described procedures may be further processed, as for example, by calendering, or other conventional processing steps commonly used in the trade.

This invention will be more fully described in conjunction with the following illustrative examples in which all parts given are by weight unless otherwise noted.

#### EXAMPLE I

This example illustrates the preparation of electroconductive paper typical of this invention by means of a procedure wherein the monoquaternary nitrogen compound is first blended with an aqueous emulsion of a polymeric coating material before its application to the paper substrate.

Two formulations were prepared containing the following components:

#### Formulation 1

154 parts of an aqueous emulsion of polyvinyl acetate having a resin solids content of 55 percent, by weight,  
35 43 parts of an aqueous solution containing 35 percent, by weight of tetramethyl ammonium chloride,  
103 parts of water.

#### Formulation 2

136 parts of an aqueous emulsion of polyvinyl acetate having a resin solids content of 55 percent, by weight, 72 parts of an aqueous solution containing 35 percent, by weight, of tetramethyl ammonium chloride,  
45 92 parts of water.

In each formulation, the aqueous solution of the tetramethyl ammonium chloride compound was diluted with the additional water and the mixture was then slowly stirred into the polyvinyl acetate emulsion.

Each of the above described formulations was applied, by means of a Meyer Wire-Wound Bar, to the sized surface of bleached sulfite paper having a basis weight of 51 pounds per ream. After the coating operation was completed, the paper was air dried for about 1 hour and then placed in an oven set at 100° C. for about 1 minute. The resulting dried coating contained the monoquaternary nitrogen compound in a concentration of about 3 pounds per ream.

Samples of the thus prepared electroconductive paper, each measuring about 2.5×3.0 inches, were cut and conditioned for about 24 hours at relative humidities of 25 and 50 percent at 72° F. The surface resistivity of each sample was determined at the specified humidity by measuring the resistance across two electrodes, spaced 0.75 inches apart on the surface of the paper, using a solid state electrometer.

Table I summarizes the results of the evaluation procedures.

TABLE I

| Sample             | Percent relative humidity | Surface resistivity, ohms/cm. <sup>2</sup> |
|--------------------|---------------------------|--------------------------------------------|
| Paper coated with— |                           |                                            |
| Formulation 1..... | 50                        | 7.5×10 <sup>7</sup>                        |
| Formulation 1..... | 25                        | 2.6×10 <sup>8</sup>                        |
| Formulation 2..... | 50                        | 5.6×10 <sup>8</sup>                        |
| Formulation 2..... | 25                        | 1.1×10 <sup>9</sup>                        |

The above data thus reveal that all of the samples had a

printing surface suitable for electroconductive printing regardless of the low relative humidity at which they had been conditioned.

#### EXAMPLE II

This example illustrates the preparation of electroconductive paper typical of this invention by means of a procedure wherein the monoquaternary nitrogen compound is applied to the paper in the form of an aqueous solution.

Part A. An aqueous solution of lauryl trimethyl ammonium chloride having a concentration of 35 percent, by weight, was tubsized onto a surface of bleached southern kraft paper having a basis weight of 48 pounds per ream. After the tubsizing was completed, the paper was dried for 1 hour and then placed in an oven set at 100° C. for about 1 minute. The resulting dried paper thus contained the lauryl trimethyl ammonium chloride in a concentration of 2.41 pounds per ream.

Part B. In a variation of the above procedure, the aqueous solution of lauryl trimethyl ammonium chloride was applied to the paper stock as used in Part A by means of a Meyer Wire-Wound Bar. The coating equipment was adjusted to provide a final dry coating of 3.57 pounds of the lauryl trimethyl ammonium chloride per ream.

Measurements of the surface resistivity of samples of each of the thus prepared electroconductive papers were then made at 72° F. and at relative humidities of 50, 35 and 15 percent, respectively. Table II summarizes the results of these determinations.

TABLE II

| Sample            | % Relative Humidity | Resistivity Ohms/cm. <sup>2</sup> |
|-------------------|---------------------|-----------------------------------|
| Paper from Part A | 50                  | $1.6 \times 10^6$                 |
| Paper from Part A | 35                  | $4.4 \times 10^6$                 |
| Paper from Part A | 15                  | $1.1 \times 10^6$                 |
| Paper from Part B | 50                  | $6.0 \times 10^6$                 |
| Paper from Part B | 35                  | $1.3 \times 10^6$                 |
| Paper from Part B | 15                  | $4.6 \times 10^6$                 |

The above data thus reveal that all of the samples had a printing surface suitable for electroconductive printing regardless of the low relative humidity at which they had been conditioned.

#### EXAMPLE III

This example illustrates the preparation of a typical coating blend containing tetramethyl ammonium chloride as the electroconductive compound along with a combination of polyvinyl acetate and a chemically derivatized starch which served as the polymeric coating component. Clay is included in the blend in order to improve the opacity of the resulting coating as well as to serve as an extender.

An aqueous emulsion of polyvinyl acetate having a resin solids content of 55 percent, by weight. 54.4 parts

A suspension of a low viscosity cationic corn starch which was prepared by treating corn starch with *b*-diethyl amino ethyl chloride hydrochloride according to the procedure described in U.S. Pat. No. 2,813,093. The suspension, which contained 15 percent, by weight, of the cationic starch, had been precooked for a period of 15 minutes at about 200° F. 200.0 parts

Clay 20.0 parts

An aqueous solution containing 35 percent, by weight, of tetramethyl ammonium chloride 52.1 parts

Water 100.0 parts

The blend was prepared by admixing the clay with the precooked starch suspension. Thereafter, the polyvinyl acetate emulsion, the aqueous solution of tetramethyl am-

monium chloride, and water were each in turn admixed with the clay-starch suspension, and the resulting blend was stirred until a homogeneous composition was obtained.

This composition was applied, by means of an air knife coater, onto bleached sulfite paper having a basis weight of 51 pounds per ream so as to yield an electroconductive paper which, after drying, contained about 3.6 pounds of tetramethyl ammonium chloride per ream. The thus prepared paper exhibited surface resistivity values which were comparable to those of the electroconductive papers whose preparation was described in Examples I and II.

#### EXAMPLE IV

15 This example illustrates the preparation and use of four coating formulations comprising blends containing varying proportions of a number of different monoquaternary nitrogen compounds and polymeric coating materials.

20 Subsequent to their preparation which was accomplished by means of the procedure described in example I, each of the formulations described below was coated, by means of an air knife coater, onto bleached sulfite paper having a basis weight of 51 pounds per ream so as to yield a coating which, after drying, contained from about 3 to 5 pounds per ream of the selected monoquaternary compound.

##### Formulation 1

An aqueous emulsion of polyvinyl acetate having a resin solids content of 55 percent, by weight. 100 parts  
An aqueous solution containing 35 percent, by weight, of dodecyl trimethyl ammonium chloride. 40 parts  
Water 90 parts.

##### Formulation 2

35 An aqueous emulsion of polyvinyl acetate having a resin solids content of 55 percent, by weight. 100 parts  
A suspension of a low viscosity, acetylated starch containing 15 percent solids, by weight. The suspension had been precooked for a period of about 15 minutes at about 200° F. 248 parts  
An aqueous solution containing 35 percent, by weight, of tetradecyl trimethyl ammonium chloride. 66 parts.

##### Formulation 3

45 An aqueous emulsion of polyvinyl acetate having a resin solids content of 55 percent, by weight. 100 parts  
An aqueous solution containing 20 percent, by weight, of polyvinyl alcohol 8 parts  
An aqueous solution containing 35 percent, by weight, of N-methyl, N-decyl pyrrolidinium bromide 70 parts.

##### Formulation 4

50 An aqueous solution containing 20 percent, by weight, of polyvinyl alcohol 100 parts  
An aqueous solution containing 35 percent, by weight, of N-hexadecyl-ethyl morpholinium ethosulfate 24 parts.

55 Each of the resulting electroconductive papers which had been prepared with the above described coating formulations exhibited surface resistivity values which were comparable to those of the electroconductive papers whose preparation was described in example I and II.

#### EXAMPLE V

65 This example illustrates the excellent conductivity achieved with a number of representative monoquaternary nitrogen compounds when used for the preparation of electroconductive papers according to the process of this invention.

Aqueous solutions of each of the compounds listed in table III, hereinbelow, were coated onto sized paper by means of a Meyer Wire-Wound Bar. On completion of the coating procedure, the various samples were air dried and then dried in an oven set at 100° C. for about 1 minute. In each case, the selected monoquaternary nitrogen compound was present in the resulting electroconductive papers in a concentration ranging from about 2 to 4 pounds per ream.

Measurements of the surface resistivity of the thus prepared samples at various relative humidities are summarized in table III.

TABLE III

| Compound                                                                  | Coating by weight, pounds/ream | Surface resistivity, ohms/cm. <sup>2</sup> at percent relative humidity |                     |                     |
|---------------------------------------------------------------------------|--------------------------------|-------------------------------------------------------------------------|---------------------|---------------------|
|                                                                           |                                | 35%                                                                     | 25%                 | 15%                 |
| 1. Stearamidopropyl trimethyl ammonium chloride                           |                                |                                                                         |                     |                     |
| 2. N-cetyl, N-ethyl morpholinium ethosulfate                              | 1.59                           | 1.7×10 <sup>7</sup>                                                     | 5.4×10 <sup>8</sup> |                     |
| 3. N-octadecylphenylmethyl, dimethyl ammonium chloride                    | 2.23                           | 7.6×10 <sup>7</sup>                                                     | 6.4×10 <sup>8</sup> |                     |
| 4. 1,2-trimethylene-1-decyl-1,4,5,6-tetrahydro-pyrimidinium bromide       | 2.08                           | 7.9×10 <sup>7</sup>                                                     | 7.4×10 <sup>8</sup> |                     |
| 5. 1,2-dimethyl-1-decyl-1,4,5,6-tetrahydro-pyrimidinium bromide           | 3.31                           | 2.9×10 <sup>7</sup>                                                     |                     | 3.4×10 <sup>8</sup> |
| 6. N-cyclohexyl trimethyl ammonium chloride                               | 3.04                           | 9.0×10 <sup>7</sup>                                                     |                     | 2.2×10 <sup>9</sup> |
| 7. Tallow (C <sub>14</sub> -C <sub>18</sub> ) trimethyl ammonium chloride | 3.26                           | 1.4×10 <sup>7</sup>                                                     | 1.1×10 <sup>8</sup> |                     |
|                                                                           | 2.45                           | 5.6×10 <sup>6</sup>                                                     | 3.9×10 <sup>8</sup> |                     |

The above data clearly demonstrate that all of the samples had a printing surface suitable for electroconductive printing regardless of the low relative humidity at which they were conditioned.

Summarizing, it is thus seen that this invention provides novel electroconductive paper products as well as a process for their preparation. Variations may be made in proportions, procedures and materials without departing from the scope of this invention which is limited only by the following claims.

What is claimed is:

1. A paper having a printing surface adapted for electroconductive printing, said paper containing at least one monoquaternary nitrogen compound selected from the group having the general formulas:



wherein R is an alkyl group containing from one to 22 carbon atoms; R' is selected from the group consisting of alkyl, aryl, aralkyl, cycloalkyl, halo-alkyl, halo-alkenyl, halo-aralkyl, HOCH<sub>2</sub>CHOHCH<sub>2</sub><sup>-</sup>, H-OCH2CH2<sub>n</sub>-OCH<sub>2</sub>CH<sub>2</sub><sup>-</sup>, and

wherein n may have a value of from 0 to 19; A is an alkylene radical containing from two to seven carbon atoms; X is an alkyl group containing from five to 15 carbon atoms; and Y is an anion selected from the group consisting of the chlorine, bromine, iodine, methosulfate and ethosulfate anions.

2. The paper of claim 1, wherein said monoquaternary nitrogen compound is present in a concentration ranging from about 0.5 to 6.0 pounds per ream of said paper.

3. The paper of claim 1, wherein said monoquaternary nitrogen compound is selected from the group consisting of:

2-undecyl-1-methyl-1-hydroxyethyl-1,4,5-dihydroimidazolinium chloride; 2-heptadecyl-1-methyl-1-hydroxypropyl-1,4,5,6-tetrahydropyrimidinium methosulfate;

N-isopentadecyl-N-trimethyl ammonium chloride; N-isoundecyl-dihydroxyethyl-methyl ammonium chloride; N'-dodecanoyl-N,N-dimethyl piperizinium chloride; N-dodecyl-methylpyrrolidinium chloride;

N-tetradecyl-methyl piperidinium chloride; 2-hydroxy-3-dodecyl benzyl trimethyl ammonium chloride; N-hexadecyl-ethyl morpholinium ethosulfate;

1,2-trimethylene-1-decyl-1,4,5,6-tetrahydropyrimidinium bromide;

N-dodecanamidopropyl-trimethyl ammonium chloride; dodecyl trimethyl ammonium chloride; tallow(C<sub>14</sub>-C<sub>18</sub>) trimethyl ammonium chloride; tallow(C<sub>14</sub>-C<sub>18</sub>) dimethyl chloro-2-butetyl ammonium chloride;

tetramethyl ammonium chloride; lauryl trimethyl ammonium chloride; tetradecyl trimethyl ammonium chloride;

N-methyl, N-decyl pyrrolidinium bromide; stearamidopropyl trimethyl ammonium chloride; N-cetyl, N-ethyl morpholinium ethosulfate; N-octadecylphenylmethyl, dimethyl ammonium chloride; 1,2-dimethyl-1-decyl-1,4,5,6-tetrahydropyrimidinium bromide; and

N-cyclohexyl trimethyl ammonium chloride.

4. The paper of claim 1, wherein said printing surface is coated with at least one coating material selected from the group consisting of: (1) polyvinyl acetate and the random copolymers of vinyl acetate; (2) polyvinyl alcohol; (3) amylaceous based materials; and (4) cellulose derivatives.

5. A process of manufacturing electroconductive paper having a printing surface adapted for electroconductive printing, comprising applying to paper at least one monoquaternary nitrogen compound selected from the groups having the general formulas:





wherein R is an alkyl group containing from one to 22 carbon atoms; R' is selected from the group consisting of alkyl, aryl, aralkyl, cycloalkyl, halo-alkyl, halo-alkenyl, halo-aralkyl,  $\text{HOCH}_2\text{CHOHCH}_2$ , H--OCH2CH2, and



wherein  $n$  may have a value of from 0 to 19; A is an alkylene radical containing from two to seven carbon atoms; X is an alkyl group containing from five to 15 carbon atoms; and Y is an anion selected from the group consisting of the chlorine, bromine, iodine, methosulfate and ethosulfate anions.

6. The process of claim 5 wherein said monoquaternary nitrogen compound is applied in a concentration ranging from about 0.5 to 6.0 pounds per ream of said paper.

about 0.5 to 0.6 pounds per ream of said paper.

7. The process of claim 5, wherein said monoquaternary nitrogen compound is selected from the group consisting of:

- 2-undecyl-1-methyl-1-hydroxyethyl-1,4,5-dihydroimidazolinium chloride;
- 2-heptadecyl-1-methyl-1-hydroxypropyl-1,4,5,6-tetrahydropyrimidinium methosulfate;
- N-isopentadecyl-N-trimethyl ammonium chloride.

N-isoundecyl-dihydroxyethyl-methyl ammonium chloride;  
 N'-dodecanoyl-N,N-dimethyl piperizinium chloride;  
 N-dodecyl-methyl pyrrolidinium chloride;  
 N-tetradecyl-methyl piperidinium chloride;  
 2-hydroxy-3-dodecyl benzyl trimethyl ammonium chloride;  
 N-hexadecyl-ethyl morpholinium ethosulfate;  
 1,2-trimethylene-1-decyl-1,4,5,6-tetrahydropyrimidinium bromide;  
 N-dodecanamidopropyl-trimethyl ammonium chloride;  
 dodecyl trimethyl ammonium chloride;  
 tallow( $C_{14}$ - $C_{18}$ ) trimethyl ammonium chloride;  
 tallow ( $C_{14}$ - $C_{18}$ ) dimethyl chloro-2-but enyl ammonium chloride;  
 tetramethyl ammonium chloride;  
 lauryl trimethyl ammonium chloride;  
 tetradecyl trimethyl ammonium chloride;  
 N-methyl, N-decyl pyrrolidinium bromide;  
 stearamidopropyl trimethyl ammonium chloride;  
 N-cetyl, N-ethyl morpholinium ethosulfate;  
 N-octadecylphenylmethyl, dimethyl ammonium chloride;  
 1,2-dimethyl-1-decyl-1,4,5,6-tetrahydropyrimidinium bromide; and  
 N-cyclohexyl trimethyl ammonium chloride.  
 The presence of the

8. The process of claim 5, wherein said printing surface is  
25 coated with at least one coating material selected from the  
group consisting of: (1) polyvinyl acetate and the random  
copolymers of vinyl acetate; (2) polyvinyl alcohol; (3)  
amylaceous based materials; and (4) cellulose derivatives.

30

35

40

45

50

55

60

65

70

75